

## UNITED STATES PATENT OFFICE

2,461,937

DEGASSING AND GRAIN REFINING OF  
MAGNESIUMKossy Strauss, Birmingham, England, assignor to  
Foundry Services Limited, Birmingham, Eng-  
land, a British companyNo Drawing. Application January 7, 1947, Serial  
No. 720,687. In Great Britain January 9, 1946

## 1 Claim. (Cl. 75—67)

**1** The present invention concerns improvements in or relating to the degassing and grain refinement of magnesium and magnesium alloys and has for its object improved means for ensuring that the agent employed for this purpose is effective over a sufficiently prolonged period of time to ensure that the process is completed.

According to the invention a solid organic chloride such as hexachloroethane is employed as the agent and is pressed into a tablet with or without the addition of reactive or inert materials so that the reaction can be prolonged and therefore the metal can be kept in contact with the gas for an extended period; preferably the tablet is thrust and held in the molten metal while the reaction is proceeding.

Furthermore, additions to the hexachloroethane which form a protective film around the hexachloroethane crystals will prolong the reaction still more. For instance hexachloroethane may be mixed with a fluoride such as sodium, potassium or magnesium fluoride or a silico-fluoride such as sodium potassium or magnesium silico-fluoride. As an example, if hexachloroethane is mixed with 20% by weight of sodium-silico-fluoride and the mixture pressed into a tablet, the sodium silico-fluoride and hexachloroethane will decompose if this tablet is plunged into the liquid magnesium. The hexachloroethane is completely volatile whilst the sodium silico-fluoride gives off silico-fluoride gas and leaves sodium fluoride as a residue. This sodium fluoride which is in intimate mixture with the hexachloroethane forms a sort of protective layer round the hexachloroethane crystals and only after the heat has penetrated completely to the core of the tablet all the hexachloroethane will have vaporized. The same effect can also be obtained by using an inert material such as asbestos powder which forms an insulating layer round the hexachloroethane crystals. In a similar way,

**2** chlorides, such as sodium chloride or potassium chloride can be used.

The vapor of hexachloroethane which is decomposed in the liquid magnesium into chlorine, carbon and organic chlorine compounds with a lower number of carbon atoms, effects the degassing and cleaning action in the metal and at the same time the carbon developed during the decomposition causes grain refinement.

**10** I claim:

The process of treating magnesium and magnesium alloys in molten state for degassing and refining the same, which consists in introducing into the melt about 20% by weight of sodium silico fluoride as an addition to hexachloroethane forming the remainder of a composition in substantially solid, compressed tablet form, and allowing said sodium silico fluoride to give off silico fluoride gas within the melt while sodium fluoride forms a residue and constitutes a protective layer around hexachloroethane crystals until the latter have completely vaporized within said melt.

KOSSY STRAUSS.

**25**

## REFERENCES CITED

The following references are of record in the file of this patent:

**30**

## UNITED STATES PATENTS

| Number    | Name         | Date          |
|-----------|--------------|---------------|
| 1,896,201 | Stern-Rainer | Feb. 7, 1933  |
| 2,378,699 | Gunn         | June 19, 1945 |

**35**

## OTHER REFERENCES

Battelle Memorial Institute, Columbus, Progress Reports on "Investigation of Cast Magnesium Alloys and of the Existing Foundry Techniques and Practices," Declassified April 23, 1946; pp. 230, 234, 398 and 399.